

May 22, 1928.

1,671,021

A. C. FISCHER

PREFORMED RAIL FILLER

Filed June 30, 1927



Inventor:  
Albert C. Fischer,  
By Ballard Moore atty

## UNITED STATES PATENT OFFICE.

ALBERT C. FISCHER, OF CHICAGO, ILLINOIS.

## PREFORMED RAIL FILLER.

Application filed June 30, 1927. Serial No. 202,578.

My invention relates to a preformed rail filler comprising a prepared strip of waterproofing material, preferably bituminous material or other suitable binder shaped to conform to the outline of the rail on one side and suitably faced for contact with the paving on the other side, the strip being adapted to act as insulating, sound deadening and expansion material, deadening the sound of the car upon the rail and insulating the track from the adjacent paving material and taking up expansion and contraction between them.

My invention is concerned more with the substance out of which the strips are made than to their particular form.

One of the objects of my invention resides in providing a preformed rail filler comprising a waterproofing binder and flakes homogeneously disposed therein, whereby not only to assist in the insulating and sound deadening characteristics of the strip, and also providing an efficient flow retarder for the compressible waterproofing binder, but also providing an efficient structural reinforcing for the rail filler, and in addition augmenting the expansibility and compressibility and sound deadening efficiency of the strip.

These and other objects of my invention will be apparent from a perusal of the following specification when taken in connection with the accompanying drawings, wherein,

Figures 1 to 6 inclusive illustrate various designs of strips which may be used singly or collectively in connection with a rail after the manner illustrated and claimed in an application filed January 6, 1926, by H. W.

Herbst, Serial No. 79,543.

It is understood that any of the blocks or strips shown in the aforesaid application, or any other type of strip may be availed of, the present invention being concerned with the material of which the rail filler strips are composed.

In the present invention I propose to form my rail filler of a homogeneous mixture of waterproofing material, such as bituminous material, preferably blown bituminous material and reinforcing flakes. These flakes may be any desired type, such for instance as, mica flakes, shale flakes, slate flakes, treated vegetable flakes, treated parchments, papier maché, and other stiffening means in flaked formation, or any type

of vegetable or mineral flakes provided they are flat and have perceptible length. Mica is well suited because of the tenacity of the flake, and the fact that the asphaltic material cannot penetrate the mica, nor would the oil be apt to affect it and destroy its stiffening quality, while the stiffening means in itself would not be subject to decay. There is also a resiliency in layer mica which might be utilized to advantage. Roasted peanut shells or flat, cellular fibrous matter is acceptable, particularly excelsior ribbon flakes, wherein the excelsior ribbon is broken up into relatively long flake-like coarseness.

In certain instances I can incorporate with the flake elements relatively long fibres which have not only length but toughness and inherent rigidity. Certain of these fibres may be cellular in nature if desired, and they are, therefore, pronouncedly compressible. The purpose of the incorporation of the cellular fibres is to secure greater re-expansibility and also to act as an additional strengthening means and to prevent the sagging of the bituminous or waterproofing binder.

The flakes, and the fibres if desired, are suitably mixed with the bituminous material when the latter is in a liquid state in a suitable power mixer, and the mixture is then preferably rolled, while plastic, according to the process set forth in an application filed January 29, 1926, Serial No. 84,605, wherein the linear fibres mixed in the plastic bituminous mass are caused to flow in the mass and align or stratify themselves lengthwise of the strip to provide stratified, overlapping, reinforcing flakes, or in other words to provide shale-like layers of the flakes within the bituminous binder, which provides not only a very pronounced reinforcing means for the strip, which gives it rigidity, acts as an efficient flow retarder for the bituminous binder, but also adds compressibility and re-expansibility and pronounced sound deadening qualities.

In certain instances where the flaked elements are of cellular nature I may mix them with the bituminous matter at a sufficiently low temperature and for a sufficiently short time to prevent the saturation of the cells of the flakes with the bituminous material, whereby the flakes retain their full compressible qualities. In other instances I contemplate mixing the cellular flakes with the bituminous material while in a suffi-

ciently heated condition and for a sufficient length of time to cause the cells of the cellular flakes to become saturated with the bituminous material.

5. The formation of my improved rail filler is somewhat the same as pieces of shale or slate which have partly separated, or resemble in the structure more or less the structure of mica itself, except that the sealing means between the flakes consists entirely of bituminous substances.

I claim:

1. A preformed rail filler adapted as an expansion joint, sound deadener and insulating material, comprising a waterproofing binder having reinforcing elements incorporated therein in the form of thin segregated flakes, each of said flakes having flat surface areas of relatively broad dimension, and 15 providing separately acting strengthening parts, the flakes being distributed thru the asphaltic material in substantially parallel strata, and the majority of the flakes being separated one from another by a substantial 20 thickness of the asphaltic material.

2. A preformed rail filler adapted as an expansion joint, sound deadener and insulating material, comprising a homogeneous 25

mixture of bituminous material and reinforcing elements in the form of segregated flakes arranged in substantially parallel strata and in overlapping relation, and separated by a bituminous substance.

3. A rail filler comprising a preformed body of bituminous material having homogeneously distributed therethru reinforcing flake-like elements arranged in substantially parallel strata, said strip also having distributed therethru linear fibres.

4. A rail filler of the character described, comprising a preformed strip of bituminous material having incorporated therein cellular flakes arranged in spaced apart stratified form and overlapping, with bituminous material between the separate flakes, said 45 flakes having their cells unpenetrated by the bituminous material.

5. A rail filler of the character described, comprising a preformed strip of bituminous material having incorporated therein cellular flakes arranged in substantially parallel strata and spaced apart, with bituminous material therebetween.

Signed at Chicago, Illinois, this 16th day of June 1927.

ALBERT C. FISCHER.